



US009708704B2

(12) **United States Patent**  
**Lapierre et al.**

(10) **Patent No.:** **US 9,708,704 B2**  
(45) **Date of Patent:** **\*Jul. 18, 2017**

(54) **METHOD FOR LOW-PRESSURE CARBONITRIDING USING A REDUCED TEMPERATURE GRADIENT IN AN INITIAL NITRIDATION PHASE**

(71) Applicant: **ECM Technologies**, Grenoble Cedex (FR)

(72) Inventors: **Philippe Lapierre**, Valentigney (FR); **Jerome Lardinois**, Courcelles les Montbeliard (FR); **Yves Giraud**, Jarrie (FR); **Alfred Rallo**, Croles (FR)

(73) Assignee: **ECM Technologies**, Grenoble (FR)

(\*) Notice: Subject to any disclaimer, the term of this patent is extended or adjusted under 35 U.S.C. 154(b) by 486 days.

This patent is subject to a terminal disclaimer.

(21) Appl. No.: **14/354,358**

(22) PCT Filed: **Oct. 8, 2012**

(86) PCT No.: **PCT/EP2012/069889**

§ 371 (c)(1),  
(2) Date: **Apr. 25, 2014**

(87) PCT Pub. No.: **WO2013/064336**

PCT Pub. Date: **May 10, 2013**

(65) **Prior Publication Data**

US 2015/0101710 A1 Apr. 16, 2015

(30) **Foreign Application Priority Data**

Oct. 31, 2011 (FR) ..... 11 59877

(51) **Int. Cl.**

**C23C 8/32** (2006.01)  
**C23C 8/02** (2006.01)

(Continued)

(52) **U.S. Cl.**  
CPC ..... **C23C 8/32** (2013.01); **C21D 1/18** (2013.01); **C22C 38/00** (2013.01); **C23C 8/02** (2013.01); **C23C 8/34** (2013.01); **C23C 8/80** (2013.01)

(58) **Field of Classification Search**  
CPC ..... C23C 8/32; C23C 8/56  
See application file for complete search history.

(56) **References Cited**

U.S. PATENT DOCUMENTS

5,273,585 A 12/1993 Shoga  
8,303,731 B2 11/2012 Berlier et al.  
(Continued)

FOREIGN PATENT DOCUMENTS

DE 102010028165 A1 10/2011  
EP 1454998 A1 9/2004  
(Continued)

OTHER PUBLICATIONS

Search report issued in PCT/EP2012/069889 on Jan. 14, 2013.  
(Continued)

Primary Examiner — Rebecca Lee

(74) Attorney, Agent, or Firm — Moreno IP Law LLC

(57) **ABSTRACT**

A method for the low-pressure carbonitriding of steel parts, in particular parts used in the manufacture of automobiles, comprises a heating step that includes a simple heating phase (M) followed by an initial nitridation phase (Ni) from a temperature between 700° C. to 750° C. to a temperature between 860° and 1000° C. and carried out using a reduced temperature gradient relative to the simple heating phase. Additionally, alternate cementing (C1-Cn) and nitridation (N1-Nn) steps are performed at constant temperature, wherein the final nitridation step is accompanied with a decrease in temperature immediately before quenching (T).

**9 Claims, 3 Drawing Sheets**



(51) **Int. Cl.**  
*C23C 8/34* (2006.01)  
*C23C 8/80* (2006.01)  
*C21D 1/18* (2006.01)  
*C22C 38/00* (2006.01)

(56) **References Cited**

U.S. PATENT DOCUMENTS

8,784,575 B2 7/2014 Berlier et al.  
2004/0250921 A1 12/2004 Yamaguchi

FOREIGN PATENT DOCUMENTS

EP 1885904 B1 12/2009  
FR 2777911 A1 10/1999  
WO 2006111683 A1 10/2006

OTHER PUBLICATIONS

Search Report issued in PCT/EP2012/069890 on Jan. 15, 2013.  
Search report issued in PCT/EP2012/069888 on Jan. 10, 2013.  
von Stark, A. et al., Handbook of Thermoprocessing Technologies:  
Fundamentals, Processes, Components, Safety, Vulkan-Verlag  
GmbH, 2005, p. 509.



Figure 1



Figure 2



Figure 3

## 1

**METHOD FOR LOW-PRESSURE  
CARBONITRIDING USING A REDUCED  
TEMPERATURE GRADIENT IN AN INITIAL  
NITRIDATION PHASE**

The present invention claims priority of French application 1159877 filed on Oct. 31, 2011 having its content (text, drawings, and claims) incorporated herein by reference.

The present invention relates to a method of low-pressure carbonitriding of steel parts, particularly, although not exclusively, parts used in the manufacturing of automobile vehicles. In particular, the invention also applies to parts used in the manufacturing of agricultural machines, machine tools, or parts in the aeronautical field.

**BACKGROUND OF THE INVENTION**

A method of low-pressure carbonitriding of steel parts comprising alternate steps of cementation and nitriding at constant temperature, preceded by a heating step and by a temperature equalization step, and followed by a quenching step, is known from document EP 1885904. As a variation, it is provided to inject a nitriding gas during the heating step and/or during the temperature equalization step, from a 800° C. temperature.

**OBJECT OF THE INVENTION**

The invention aims at improving the method of the previously-mentioned document, that is, at improving the quality of the obtained parts, preferably with a decrease of the treatment time.

**BRIEF DESCRIPTION OF THE INVENTION**

To achieve this aim, the present invention provides a method of low-pressure carbonitriding of steel parts, particularly parts used in the manufacturing of automobile vehicles, comprising alternate steps of cementation and nitriding at constant temperature, preceded by a heating step comprising a simple heating phase followed by an initial nitriding phase while carrying on the heating, and followed by a quenching step, wherein during the initial nitriding phase, the heating is carried out with a decreased temperature gradient as compared with the simple heating phase.

Thus, the parts are maintained for a longer time in a temperature range promoting a good nitriding.

According to an advantageous version of the invention, the initial nitriding phase comprises a temperature stage.

Thus, the initial nitriding phase is carried out in optimal temperature conditions, so that it is possible to shorten or to suppress one of the subsequent nitriding steps at the cementation temperature, and to thus decrease the total treatment time.

According to another advantageous aspect of the invention, the initial nitriding phase is immediately followed by a first cementation step. Thus, the total suppression of the temperature equalization phase enables to lengthen the initial nitriding phase in a temperature range optimal for nitriding.

According to another advantageous aspect of the invention, the method comprises a step of final nitriding accompanied by a cooling immediately before the quenching. Preferably, the final nitriding step comprises a temperature stage. Thus, the final nitriding step is also carried out in an optimal temperature range, so that the quality of the treatment is improved.

## 2

**BRIEF DESCRIPTION OF THE DRAWINGS**

The foregoing and other objects, features, and advantages will appear on reading of the following description of 5 different specific non-limiting embodiments of the low-pressure carbonitriding method according to the invention, in relation with the 3 appended drawings, which are simplified diagrams illustrating the different steps of the method according to the invention according to different embodiments.

**DETAILED DESCRIPTION OF THE  
INVENTION**

15 Referring to FIG. 1, the method according to the invention comprises a first heating step comprising a first simple heating phase M, illustrated by a continuous straight line, from the ambient temperature to a point at a 700° C. temperature, noted Ni1 in the drawing. According to the 20 composition of the steel to be treated, the simple heating phase may be carried out until a temperature in the range from 700° C. to 750° C. is reached, and has a duration in the range from 10 min to 90 min, that is, the simple heating is carried out with a temperature gradient in the range from 8° C./min to 75° C./min.

The method then comprises an initial nitriding phase Ni during which the heating step is carried on up to a 940° C. temperature in the illustrated example. In practice, the 940° C. temperature corresponds to a compromise between a 860° 30 C. temperature, which enables to achieve a treatment of better quality and a 1,000° C. temperature, which enables to perform a faster treatment.

In the embodiment of FIG. 1, corresponding to a first embodiment of the initial nitriding phase, the heating carries 35 on regularly but with a temperature gradient in the range from 3.5° C./min and 16° C./min, smaller than the temperature gradient during the simple heating. The initial nitriding phase lasts for from 15 min to 45 min, according to the quantity of nitrogen which is desired to be fixed in this initial 40 step and to the composition of the steel to be treated.

As known per se, the initial nitriding phase comprises phases of injection of a nitriding gas such as ammonia alternating with diffusion phases.

According to a second embodiment of the initial nitriding 45 phase, illustrated in FIG. 2, the heating carries on with the same temperature gradient as during the simple heating up to a point at a temperature in the range from 750° C. to 850° C., here 800° C., noted Ni2 in FIG. 2. The temperature is then maintained at a stage until a time noted Ni3 in FIG. 2 50 from which a strong heating is achieved to reach the cementation temperature. The stage temperature is selected in a way known per se to perform the initial nitriding phase in optimal conditions given the composition of the parts to be treated. It should be noted, on this regard, that given the stage, the final heating may be carried out very rapidly, for 55 example from 80° C./min to 100° C./min, without submitting the parts to unacceptable stress.

According to a third embodiment of the initial nitriding phase, illustrated by means of FIG. 3, the heating carries on 60 from point Ni1 with a lower temperature gradient than in the first embodiment, preferably in a range from 2° C./min to 8° C./min, until a time noted Ni4, here corresponding to a 850° C. temperature, from which a strong heating is achieved to reach a cementation temperature, according to a gradient 65 similar to that of the second embodiment.

Whatever the embodiment used for the initial nitriding phase, the method then comprises n cementation phases

alternating with nitriding phases. As known per se, the cementation and nitriding steps comprise phases of injection of a treatment gas alternating with diffusion phases, not shown in the drawings. In the drawing, the diagram has been interrupted between nitriding step N1 and last cementation step Cn. At the end of this last cementation step Cn, the method comprises a final nitriding step Nn accompanied by a cooling immediately before quenching T.

According to a first embodiment of last nitriding step Nn, illustrated by a short-dashed line in the drawing, the cooling is achieved continuously down to a temperature in the optimal temperature range for the nitriding while remaining sufficiently high to allow an efficient quenching. In the illustrated example, the final temperature before quenching is 840° C. In practice, satisfactory results are obtained for a final temperature before quenching in the range from 900° C. to 800° C. It has been observed that such a limited temperature decrease the stress on parts during the quenching.

The final nitriding step has a duration preferably between 15 min and 60 min, which corresponds to a temperature gradient in the range from 10° C./min to 1° C./min. In the same way as for the initial nitriding phase, the final nitriding step preferably comprises phases of injection of a nitriding gas alternating with diffusion phases.

According to a second embodiment of last nitriding step Nn, illustrated in FIG. 2, the cooling is first very strong, with as large a gradient as possible without generating undue stress in the steel down to the optimal nitriding temperature for the steel being treated, noted Nn1 in the drawing, here 840° C., after which the temperature is maintained at a stage until the beginning of the quenching.

In practice, the method according to the invention may be implemented by combining any of the embodiments of the initial nitriding phase with any of the embodiments of the final nitriding phase, or even ending the treatment cycle conventionally, that is, with a quenching performed directly from the cementation temperature.

It should be noted that due to the increased efficiency of the nitriding phases according to the invention, it is possible to replace at least one nitriding step comprised between two cementation steps with a simple diffusion step. Such a step is shorter than a nitriding step so that the total duration of the treatment is shortened.

Of course, the invention is not limited to the described embodiment and alternative embodiments may be applied thereto without departing from the framework of the invention such as defined in the claims. In particular, although the invention has been described in relation with an initial nitriding phase starting in a temperature range from 700° C. to 750° C., it may be provided to start it only when the parts have reached an optimal nitriding temperature.

Due to the small temperature gradient during the initial nitriding phase, it has been experienced that the temperature of the parts to be treated has time to equalize so that it is possible to suppress the equalizing step provided in the previously-mentioned document. If necessary, for example, due to a specific configuration of the parts to be treated, a short temperature equalization step may however be provided between the initial nitriding phase and the first cementation phase.

10 The invention claimed is:

1. A low-pressure carbonitriding method of steel parts comprising alternate cementation and nitriding steps at constant temperature, preceded by a heating step comprising a simple heating phase followed by an initial nitriding phase during which the heating is carried on, and followed by a quenching step, wherein during the initial nitriding phase, the heating is performed with a decreased temperature gradient as compared with the simple heating phase.

20 2. The low-pressure carbonitriding method of claim 1, wherein the initial nitriding phase comprises a temperature stage.

25 3. The low-pressure carbonitriding method of claim 1, wherein the initial nitriding phase is carried out with a temperature gradient in the range from 3.5° C./min to 16° C./min.

30 4. The low-pressure carbonitriding method of claim 1, wherein the simple heating phase is carried out with a temperature gradient in the range from 8° C./min to 70° C./min.

35 5. The low-pressure carbonitriding method of claim 1, wherein the initial nitriding phase is carried out from a temperature between 700° C. and 750° C., and up to a temperature between 860° C. and 1,000° C.

40 6. The low-pressure carbonitriding method of claim 1, wherein the initial nitriding phase is immediately followed by a first cementation step.

45 7. The low-pressure carbonitriding method of claim 1, further comprising a final nitriding step accompanied by a cooling immediately before the quenching, wherein the cooling is achieved down to a temperature between 900° C. and 800° C.

50 8. The low-pressure carbonitriding method of claim 1, further comprising a final nitriding step accompanied by a cooling immediately before the quenching, wherein the cooling is carried out with a temperature gradient between 10° C./min and 1° C./min.

9. The low-pressure carbonitriding method of claim 1, further comprising a final nitriding step accompanied by a cooling immediately before the quenching, wherein the final nitriding step comprises a temperature stage.

\* \* \* \* \*